

Patented Aug. 27, 1929.

1,726,194

# UNITED STATES PATENT OFFICE.

WILHELM SANDER, OF ESSEN-RUHR, GERMANY, ASSIGNOR TO THE FIRM OF TH. GOLDSCHMIDT A.-G., OF ESSEN, GERMANY.

## PROCESS OF IMPROVING ALUMINUM ALLOYS.

No Drawing. Application filed January 19, 1928, Serial No. 248,007, and in Germany January 20, 1927.

This invention relates to a process of improving aluminum alloys; and it comprises a method of improving the properties of a special alloy containing certain minor proportions of magnesium silicid, copper, titanium and, usually, manganese, wherein such an alloy is mechanically worked, is subjected to heat treatment at 520 to 550° C., is rapidly cooled and is thereafter aged at an elevated temperature; all as more fully hereinafter set forth and as claimed.

It is customary to alloy aluminum with various other metals and substances in order to improve its physical and mechanical properties. Magnesium is a frequent alloying constituent and in addition heavy metals may be present. In some aluminum alloys magnesium is replaced by magnesium silicid; a substance which is very useful. In this type of aluminum alloys the relative proportion of the silicon is such as to form the compound  $Mg_2Si$  without excess of either magnesium or silicon. These alloys containing magnesium silicid also have been improved by the addition of heavy metals and particularly copper. In practical use however these copper-containing alloys are not all that can be desired. Increasing the copper content brings an increase in strength but lessens the suitability for cold and hot working. There is a reduction in the expansion and an increased corrodibility. Lowering the copper content to avoid these difficulties makes the strength of the alloy too low.

In the prior Patent No. 1,656,502, January 17, 1928, whereon the present invention is in some aspects an improvement, a particularly desirable alloy was described, this alloy carrying magnesium silicid, 1.2 per cent copper and a little titanium. In the present invention an alloy of this type is employed. As the result of exhaustive investigation of alloys of this type it is found that the best results are obtained with certain rather special ratios between the alloying bodies and the aluminum and between these components themselves and a special method of working this alloy has been developed. With this composition and this method of working it is possible not only to secure maximum tensile strength, elongation and suitability for

hot and cold working but also good resistance to chemical action.

An alloy of the following composition

|                    |                        |    |
|--------------------|------------------------|----|
| Mg <sub>2</sub> Si | 1.5 per cent $\pm$ 0.2 | 55 |
| Copper             | 1.2 per cent $\pm$ 0.2 | 60 |
| Titanium           | 0.5 per cent $\pm$ 0.2 | 65 |

exhibits an extremely good relationship between strength, elongation, suitability for hot and cold working and resistance to corrosion. An addition of a slight amount of manganese still further improves the alloy; this giving an increase in strength and rendering the alloy insensitive to superheating. 65 In the presence of the manganese it is not necessary to maintain an exact temperature in annealing between stages of working as with other alloys. The range of temperatures within which intermediate annealing 70 can be successfully carried out is considerably increased. As a rule, 0.8 per cent of manganese, with a plus or minus variation of 0.3 per cent, gives the best results.

With this alloy, the best method of working as yet devised in obtaining good mechanical strength includes a preliminary mechanical working, for example by rolling, drawing, pressing or forging. After this working the alloy is raised to 520 to 550° C. in 80 about half an hour, and then rapidly cooled, cooling being followed by an ageing operation at an elevated temperature. The best temperatures are between 110 and 150° C. with a treatment period of about 6 to 24 85 hours. There is a choice as to these temperatures. Low annealing temperatures and short annealing times give a material with a particularly high elongation while on the other hand a prolonged annealing at high 90 temperatures gives a material of particularly high strength with good elongation.

In the event that high requirements are made as to elongation and resistance to corrosion, it has been found beneficial to begin 95 the ageing treatment at the high temperature after a preliminary rest at room temperature, this resting period following the cooling. A rest period of 24 to 48 hours at room temperature is generally sufficient. 100 After the resting period the ageing at the high temperature is resorted to. In the

- event of special requirements in regard to strength, it has been found that high strengths can be imparted by interposing another mechanical working following the first high temperature treatment and the subsequent cooling. After this, the procedure is as before. Special results as regards strength, elongation, resistance to corrosion etc. can be obtained with variations in the described procedure consisting in using mechanical working at different stages in the operation, after annealing, after cooling, or after different time intervals prior to the intermediate rest at room temperature.
- Material of the stated composition treated in the stated manner gives a tensile strength of 37 to 54 kilograms per square millimeter with an elongation of 28 to 12 per cent. Corrosion tests show only about half the corrodibility of ordinary aluminum alloys. The material has excellent cold bending properties. Sheets and wires can be bent in an arc of very small radius. For example, a 4-millimeter sheet having a tensile strength of 41 kilograms per square millimeter can be bent by hammering through 180° round a radius of 7 to 8 millimeters. This malleability is about double that of the known aluminum alloys of the same tensile strength. Not only is the malleability in the cold good but the malleability with a hot working is excellent. The present material can be easily pressed and drawn into thin tubes and complicated contours without requirement of frequent intermediate annealings and small intermediate stages of reduction. This fact gives great economy in the use of the present material.
- Still higher strengths, though with sacrifice of elongation, can be obtained by submitting the material to a final mechanical treatment.
- What I claim is:—
1. In the improvement of alloyed aluminum containing 1.3 to 1.7 per cent magnesium silicid, 1 to 1.4 per cent copper, and 0.3 to 0.7 per cent titanium, with or without 0.5 to 1.1 per cent manganese, the process which comprises mechanically working a body of said alloy, heat treating at 520° to 550° C., rapidly cooling and subsequently ageing at a temperature higher than room temperature.
  2. In the improvement of alloyed aluminum containing 1.3 to 1.7 per cent magnesium silicid, 1 to 1.4 per cent copper, and 0.3 to 0.7 per cent titanium, with or without 0.5 to 1.1 per cent manganese, the process which comprises mechanically working a body of said alloy, heat treating at 520° to 550° C., rapidly cooling and subsequently ageing at a temperature between 110° and 150° C. for 6 to 24 hours.
  3. In the improvement of alloyed aluminum containing 1.3 to 1.7 per cent magnesium silicid, 1 to 1.4 per cent copper, and 0.3 to 0.7 per cent titanium, with or without 0.5 to 1.1 per cent manganese, the process which comprises mechanically working a body of said alloy, heat treating at 520° to 550° C., rapidly cooling and subsequently ageing at a temperature between 110° and 150° C. for 6 to 24 hours, the alloy body being allowed to rest for a time prior to applying the ageing treatment.

In testimony whereof I affix my signature.

WILHELM SANDER.